

## UNITED STATES PATENT OFFICE

2,229,923

DECORATION OF TEXTILE AND OTHER  
TISSUESEric Berkeley Higgins, Punchetts, Tewin Wood,  
EnglandNo Drawing. Application May 24, 1938, Serial No.  
209,849. In Great Britain May 28, 1937

13 Claims. (CL 8—17)

This invention relates to the coloring and decoration of textile and like materials, especially fabrics and yarns, and is particularly concerned with the production of colored, waterproofed materials.

In co-pending United States application, Serial No. 205,818 filed May 3rd, 1938, there is described a process for waterproofing textile materials by causing an amphoteric protein to react on the materials under acid conditions with a compound containing an amphoteric metal.

It has now been found that if the reaction is effected in the presence of a coloring matter, products which are both colored and waterproofed are obtained, and, moreover, that on dyeing by means of the process the shades developed are deeper than would be obtained by dyeing with the same amount of dyestuff by ordinary dyeing methods.

According to the invention, therefore, colored waterproofed materials are produced by causing an amphoteric protein and a compound containing an amphoteric metal to react together on textile and like materials under acid conditions in the presence of a coloring matter.

The protein employed may, for instance, be casein, and examples of suitable amphoteric metal compounds are compounds of zinc and aluminum, for instance hydrated oxides. Aluminates may be employed, and where the acid used to bring about reaction is applied in conjunction with the metal compound, such compounds as aluminum hexaacetate or hexaformate may be employed.

The protein, metal compound and acid may be introduced in any suitable way, provided that reaction under acid conditions takes place on the material being treated, and one method of carrying out the invention is to impregnate the materials with a solution of an amphoteric protein in a neutral or alkaline medium, remove excess liquor by pressure, suction or centrifugal force, and then to treat the materials with the metal compound, in which case reaction takes place very rapidly. The acid may be applied together with the metal compound, for instance by applying an acid solution of the compound, or may be applied subsequently, for instance by immersing the materials in an acid bath or by treating them with a volatile acid. Another method of carrying out the invention is to apply the protein and the metal compound together in a neutral or alkaline medium, and then treat the impregnated materials with acid.

Yet another method of carrying out the proc-

ess of the invention is to apply to the materials, separately or together with the protein, metal compound or both, a substance which during the course of the process develops acidity and causes reaction to take place. Examples of such substances are ammonium or pyridinium salts of organic acids. Such salts on drying decompose with evaporation of the base, leaving free acid. In this case, reaction will take place on drying the treated materials.

After the reaction, excess acid on the materials is preferably removed, for instance by washing, or, where the acid is volatile, by volatilisation.

The coloring matter may be applied in any suitable manner, and may for instance be applied in conjunction with the protein or the metal compound, or incorporated in the mixture of the two reagents where they are applied together. The coloring matter may, for example, be an acid, direct or basic dyestuff, or an insoluble pigment. Again, developed colors may be employed, for instance azoic colors derived from the arylides of 2,3-hydroxynaphthoic acid. Thus the arylide may be dissolved in an alkaline solution of the protein and metal compound, the resultant solution applied to the material being treated, and the materials subsequently treated with an acetic acid solution of the diazotised amine with which the arylide is to be developed. In this case the acetic acid solution will effect both development of the dyestuff and reaction between the protein and the metal compound.

Which of the various alternative methods of carrying out the process of the invention is to be used in any given case will depend upon the material treated.

The amphoteric protein is preferably applied to the materials in an alkaline solution having a pH value of about 10, although lower pH values, for instance about 8, may also be employed, especially if buffer salts such as borax or soap are present. The acidity at which the reaction between the protein and the amphoteric metal is effected is suitably that of a pH value between 3.5 and 6.5, and it follows that in certain cases the acid medium may even be the carbon dioxide of the atmosphere, although pH values lower than 6-6.5 are to be preferred.

Alkaline solutions of amphoteric proteins are in general compatible with alkaline soaps, and where an alkaline solution of an amphoteric protein containing if desired the amphoteric metal compound is being employed, alkaline soaps may be incorporated therein. Again, alkaline solu-

10

15

20

25

30

35

40

45

50

55

tions of amphoteric proteins, whether an alkaline 5 soap is present or not, possess excellent emulsifying and wetting properties, and fats, waxes and similar materials may be emulsified in the solutions. Thus fats, waxes and the like may be present on the materials being treated when reaction takes place, and it has been found that by this means additional water-repelling properties, as 10 distinct from waterproof properties, may be obtained, at least temporarily.

In practice, the full waterproofing effect of the process is not shown until the metal-protein compound produced has been "dehydrated," this taking place on drying the material, if desired 15 at atmospheric temperature. Low temperature drying is especially valuable where delicate fabrics are being treated, for instance fabrics of the "substitute" type, e. g. paper composites, or fabrics containing cellulose acetate threads, 20 which are liable to be damaged at high temperatures.

The alkaline solutions of protein containing coloring matter which may be used according to the invention are suitably prepared in a concentrated 25 form and diluted for use. The concentrated solutions are well fitted for storage.

A suitable method of carrying out the process of the invention is to dissolve or suspend the coloring matter in a solution of the amphoteric 30 protein or the metal compound, or in a solution of both reagents, and to pad, dye, print, stencil or spray fabric or yarn with the product, reaction being subsequently effected as described above. By the adoption of such a treatment not only is 35 the self dyed or printed effect accomplished with a great saving of coloring matter and at a vastly higher speed than is usual by ordinary methods of coloring, but the dyer or printer is rendered completely or almost completely independent 40 of the specific properties which usually confine certain coloring matters to certain fabrics. The reaction may be carried out practically in the cold, and without the necessity of special preparation of the fabric. Thus, for example, 45 fabrics imported from the East or elsewhere, e. g. Japanese silks, may be colored without necessarily removing the manufacturer's finish, and consequently many expensive operations now necessary in the coloring of such imported products 50 may be eliminated.

The method of application should be varied in accordance with the type of dyeing or printing to be adopted. In general, for self-colored goods the most advantageous method is to pad the 55 goods in open width through a protein-metal compound-color mixture, remove the excess of the mixture by rollers or by suction, run the impregnated cloth in open width into the acidifying solution, for example a 1-6% solution of acetic, 60 formic or oxalic acid, and then after removal of excess liquor to run the cloth through water to remove the remaining free acid. The material is then dried and finished. If a volatile acid is employed the fabric may be dried direct and the 65 washing operation omitted. In this manner a silk fabric, for example, may be dyed an even shade of an acid color equivalent in intensity at least to that obtained by a double amount of the same color dyed in the ordinary way upon the 70 same cloth. Moreover, if desired the treatment may be carried out at atmospheric temperature and continuously at a rate up to 120 to 130 linear yards per minute. The same acid color may be applied in the same way to yarns or fabrics, woven or knitted, of cotton, linen, viscose 75

or acetate rayon, wool or, indeed, to any yarns or fabrics, though as is well known many of these materials are not dyed at all by acid colors by the ordinary processes of dyeing. Similarly, basic or direct colors may be applied to all types of 5 fabrics and yarns independently of their substantivity or otherwise. It is also possible to attach insoluble colors and pigments to the fibre similarly, for instance by suspending them in a protein-metal mixture which is applied to the 10 materials being treated.

Since by the treatment the materials are colored and waterproofed simultaneously, they do not bleed in water, notwithstanding the lack of substantivity of the color to the fibre in some 15 cases. Moreover the materials will endure cleaning with volatile solvents such as white spirit or benzene.

Where it is desired to color a portion only of a material, as for instance in printing, by roller, 20 block, stencil or screen, or aerograph or by any of the recognised methods employed, it is advantageous in general to cause the necessary acid conditions to be set up either by passing the material after it has been printed with an alkaline 25 protein-metal compound-color medium through acid vapor or through acidified steam, acidified for example with acetic acid, or to incorporate in the printing paste bodies which, when the printed material is dried, will generate by their 30 decomposition the necessary acid.

The invention is illustrated by the following examples:

#### Example 1

7½ lbs. of oleic acid are mixed with 7½ lbs. of hard paraffin scale, and the mass is treated with a quantity of strong caustic soda solution (for instance a 20% solution) sufficient to convert the oleic acid into soap. A solution of 8¼ lbs. of casein and 2½ lbs. of borax in 45 lbs. of water is then added in a steady stream with continuous stirring. The homogeneous product is diluted with water to 100 lbs. weight, when a homogeneous cream very suitable for storage is obtained. 10 lbs. of this cream are diluted with 140 lbs. of a 1% solution of an acid dyestuff, e. g. Naphthalene Red, or a direct dyestuff, e. g. Benzo Sky Blue, or of a ¼% solution of a basic dyestuff, e. g. Methylene Blue DBB, and the mass is mixed to give a homogeneous solution. Through this solution a cloth, for instance of silk, wool or cotton, is padded, preferably in a three-roll padding machine of the usual construction. A high velocity of treatment, for instance up to 120 linear yards per minute, may be employed. On emerging from the padding machine, in which excess of liquor has been removed from the treated materials, so that they contain about their own weight of liquor, the materials are passed directly in open width through a second padding machine, where they come into contact with a solution of aluminium hexaacetate or hexaformate of about ½<sub>15</sub> N. strength, this solution being if desired rendered slightly more acid by the addition of 65 acetic or formic acid. From this padding machine the goods are passed directly through a drying stenter.

The finished product possesses water-repelling properties, and the shade developed is more intense than would have been obtained by dyeing with the same amount of dyestuff in the usual manner.

#### Example 2

7½ lbs. of tallow fatty acids are mixed with 6 75

lbs. of paraffin scale, and the mass is treated with concentrated aqueous caustic potash. While the soap produced is still molten, a solution of 10 lbs. of casein and 3 lbs. of decahydrated borax in 100 lbs. of water is added with stirring, and when a homogeneous liquor has been formed it is allowed to cool. 3.36 lbs. of sodium aluminate (52 to 53%  $Al_2O_3$ , 42.5%  $Na_2O$ ) are then mixed with the mass, and a product in a satisfactory condition for storage and having a pH value of 10 or more is obtained. 10 lbs. of this product are then mixed with 140 lbs. of dyestuff solution, e. g. a  $\frac{1}{4}\%$  solution of an acid or direct dyestuff or a  $\frac{1}{8}\%$  solution of a basic dyestuff, and textile materials are padded in a padding machine with the liquor produced. After leaving the padding machine the goods are run into a  $\frac{1}{15}$  N. solution of acetic or formic acid and are then dried on a stenter in the usual manner.

The intensity of shade so developed is equal to that developed by at least three times the quantity of dyestuff when this dyestuff is applied by the usual methods of dyeing.

*Example 3*

The paste produced as described at the beginning of Example 2 and referred to as having a pH value of 10 or more is mixed with a solution of an acid, direct or basic dyestuff in the proportions of two parts of the paste to one of dyestuff solution. The dyestuff solution may suitably be of such a concentration that the product contains, for example, 1% of an acid or direct dyestuff or  $\frac{1}{4}\%$  of a basic dyestuff. The mixture produced is used directly as a printing paste for the production of screen prints upon Japanese silk web in its raw state as received by the importer. The screen printed piece is passed directly after printing through a low pressure steamer, in which the steam vapor has been rendered acid by the introduction of a volatile acid such as acetic or formic acid, the temperature being such that the goods do not become wet. From this steamer the goods are passed at once to drying and calendering.

The intensity of shade so developed is equal to that developed by at least three times the quantity of dyestuff employed when the goods are dyed by normal processes.

*Example 4*

8.25 lbs. of casein are mixed with 2.5 lbs. of decahydrated borax and the mixture is fed with constant stirring into 90 lbs. of water. When the mass is homogeneous, 15 lbs. of commercial soap flakes are added slowly and the stirring is continued, water being added until the whole mass weighs about 100 lbs. and is homogenous. The mixture is then cooled or allowed to cool, preferably with stirring, and a solution of 4 lbs. of sodium aluminate in 40 lbs. of water is added. When the product is cold, a solution of 15 lbs. of pyridine oxalate or acetate or ammonium oxalate or acetate in 400 lbs. of water is added. The paste obtained is mixed with a solution of an acid, direct or basic dyestuff in the proportions two parts of paste to one of solution, the solution of dyestuff being sufficiently concentrated to give a final mix containing for example 1% of an acid or direct dyestuff or  $\frac{1}{4}\%$  of a basic dyestuff.

The product is employed for block printing calico in the usual way. After printing, the pieces are immediately dried, for instance on

"tins" at a steam pressure of 10 lbs. per square inch gauge, or in a stove.

The heating step completes the operation, and the colored product possesses at least three times as deep a shade as would be produced with the same amount of dyestuff used in ordinary processes. In addition, the pattern is waterproof.

*Example 5*

To 10 lbs. of the product obtained in the manner described at the beginning of Example 4, after the addition of the pyridine oxalate or acetate or ammonium oxalate or acetate, there are added 140 lbs. of a 1% solution of an acid dyestuff, e. g. Naphthalene Red, or a direct dyestuff, e. g. Benzo Sky Blue, or of a  $\frac{1}{4}\%$  solution of a basic dyestuff, e. g. Methylene Blue DBB, and the mass is mixed to give a homogeneous solution. Through this solution a cloth, for instance of silk, wool or cotton, is padded, preferably in a three-roll padding machine of the usual construction. A velocity of treatment up to 120 linear yards per minute may be employed. On emerging from the padding machine, in which excess of liquor has been removed from the treated materials, so that they contain about their own weight of liquor, the products are passed in open width to drying tins supplied with steam at a pressure of 10 lbs. per square inch gauge, or to a stove, and are dried.

*Example 6*

To the 100 lbs. of homogeneous cream produced as described at the beginning of Example 1 are added  $1\frac{1}{2}$  lbs. of an arylide of 2,3-hydroxy-naphthoic acid, for instance the anilide sold under the registered trade-mark "Brenthol A. S." and the materials are well pasted together. To this paste is added 1,400 lbs. of water at a temperature of about 40° C., the addition being made gradually and the paste being worked to give as homogeneous a product as possible. Cotton cloth is padded through such a mixture, for instance through a three-roll padding machine, preferably to give a product containing about its own weight of liquor. The goods are then passed in open width to a second padding machine containing the customary developing solution, for instance a solution of diazotised m-nitro-p-toluidine in an equivalent concentration to that of the arylide in the first bath, there having been added to the developing solution sufficient aluminium hexaformate or hexaacetate to form in the diazo solution a  $1/15$  N. concentration of the hexa salt. The goods on leaving the developing bath are run in open width through a washing machine, and are dried, stentered and finished in the usual way.

The color so produced is especially fast to rubbing. This is a great advantage, for it is well known that colors of the hydroxynaphthoic acid arylide group are normally unsatisfactory when subjected to rubbing.

I claim:

1. A process for the production of colored, waterproofed textile and like materials, which comprises causing an extremely dilute solution of an amphoteric protein to react in the cold with an extremely dilute solution of a compound containing an amphoteric metal on the material under acid conditions and in the presence of a coloring matter to develop an insoluble colored complex within the fibre.

2. A process for the production of colored, waterproofed textile and like materials, which

comprises impregnating the individual fibres of the material in the cold with a non-acid solution of an amphoteric protein and causing the protein to react with a solution of a compound containing an amphoteric metal on the material and under acid conditions and in the presence of a coloring matter to develop an insoluble colored complex within the fibre.

5 3. A process for the production of colored, 10 waterproofed textile and like materials, which comprises impregnating the individual fibres of the material in the cold with a non-acid solution of an amphoteric protein and then treating the impregnated material, in the presence of a coloring matter, with an acid solution of a compound containing an amphoteric metal, to develop an insoluble colored complex within the fibre.

4. A process for the production of colored, 20 waterproofed textile and like materials, which comprises impregnating the individual fibres of the material in the cold with a non-acid solution of an amphoteric protein, treating the impregnated material with a non-acid solution of a compound containing an amphoteric metal, and 25 then rendering the material acid in the presence of a coloring matter, to develop an insoluble colored complex within the fibre.

5. A process for the production of colored, 30 waterproofed textile and like materials, which comprises impregnating the individual fibres of the material in the cold with a non-acid solution of an amphoteric protein and a compound containing an amphoteric metal, said solution containing a coloring matter, and then rendering 35 the impregnated material acid, to develop an insoluble colored complex within the fibre.

6. A process for the production of colored, 40 waterproofed textile and like materials, which comprises impregnating the individual fibres of the material in the cold with a non-acid solution of casein containing a coloring matter, and then treating the impregnated material with an acid 45 solution of a compound containing an amphoteric metal, to develop an insoluble colored complex within the fibre.

7. A process for the production of colored, 50 waterproofed textile and like materials, which comprises impregnating the individual fibres of the material in the cold with an alkaline solution of casein of a pH value of about 10, containing a coloring matter, and then treating the impregnated material with an acid solution of a compound containing an amphoteric metal, to

develop an insoluble colored complex within the fibre.

8. A process for the production of colored, 5 waterproofed textile and like materials, which comprises impregnating the individual fibres of the material in the cold with an alkaline solution of casein and causing the casein to react with an aluminate on the material under acid conditions and in the presence of a coloring matter to develop an insoluble colored complex within the 10 fibre.

9. A process for the production of colored, 15 waterproofed textile and like materials, which comprises impregnating the individual fibres of the material in the cold with an alkaline solution 15 of casein and causing the casein to react with an organic aluminum salt on the material in the presence of a coloring matter to develop an insoluble colored complex within the fibre.

10. An impregnated textile material having 20 developed within the fibre so much of an insoluble colored complex containing a coloring matter and the product of the reaction between an amphoteric protein and a compound containing an amphoteric metal, that the material is colored 25 and rendered waterproof but substantially retains the remaining initial qualities of the material as such.

11. An impregnated textile material having 30 developed within the fibre so much of an insoluble colored complex containing a coloring matter and the product of the reaction between casein and a compound containing an amphoteric metal, that the material is colored and rendered waterproof but substantially retains the remaining initial qualities of the material as such.

12. An impregnated textile material having 35 developed within the fibre so much of an insoluble colored complex containing a colored matter and the product of reaction between casein and aluminium hexa-formate, that the material is colored 40 and render waterproof but substantially retains the remaining initial qualities of the material as such.

13. An impregnated textile material having 45 developed within the fibre so much of an insoluble colored complex containing a coloring matter and the product of reaction between casein and an aluminate, that the material is colored 50 and rendered waterproof but substantially retains the remaining initial qualities of the material as such.

ERIC BERKELEY HIGGINS.